

[54] PRODUCTION OF STAIN RESISTANT,  
CLEAR, SEALED ANODIZED FILMS[75] Inventors: Kenneth E. Weber, Granada Hills;  
Donald G. Crozier, Burbank; Wilbur  
W. Hawley, Santa Ana, all of Calif.[73] Assignee: Lockheed Aircraft Corporation,  
Burbank, Calif.; by said Weber and  
Crozier

[22] Filed: Sept. 5, 1972

[21] Appl. No.: 286,595

[52] U.S. Cl..... 204/35 N

[51] Int. Cl..... C23c 7/00

[58] Field of Search..... 204/35 N

## [56] References Cited

## UNITED STATES PATENTS

|           |         |               |          |
|-----------|---------|---------------|----------|
| 2,888,388 | 5/1959  | Stiller.....  | 204/35 N |
| 3,257,244 | 6/1966  | Barkman.....  | 204/35 N |
| 3,616,298 | 10/1971 | Fassell ..... | 204/35 N |
| 3,704,210 | 11/1972 | Patrie.....   | 204/35 N |

Primary Examiner—John H. Mack

Assistant Examiner—R. L. Andrews

Attorney, Agent, or Firm—George C. Sullivan; Lowell  
G. Turner

## [57] ABSTRACT

A stain resistant, substantially clear, anodized aluminum coating may be produced by: anodizing an aluminum body or article in a conventional manner such as in a sulfuric acid electrolyte; rinsing the anodized film produced; partially sealing this anodized film by contacting this film with a solution containing from about 0.1% to about 5% by weight chromic oxide either present as chromic acid or as a soluble salt of this acid and from about 0.5% to about 10% by weight of a soluble tungstate salt having a pH of from about 4.5 to about 8.0 at a temperature of from about 130°F. to immediately below the boiling point of the solution; and then finally sealing this partially sealed anodized film by contacting it with a solution containing from about 0.1% to about 10% by weight of a soluble nickel or cobalt salt of a weak acid, preferably an acid selected from the group consisting of boric, citric, formic and acetic acid having a pH of from about 4.5 to about 8 at a temperature of from about 150°F. to immediately below the boiling point of the solution. Preferably the final sealing solution is buffered so that its pH will be maintained within this range.

15 Claims, 1 Drawing Figure



## ANODIZE AN ALUMINUM OBJECT

TO PRODUCE AN  
ANODIZED COATING



PARTIALLY "CLEAR SEAL" THE ANODIZED COATING BY  
CONTACTING IT WITH AN AQUEOUS SOLUTION  
CONTAINING FROM ABOUT 0.1% TO ABOUT 5%  
BY WEIGHT CHROMIC OXIDE AND FROM ABOUT  
0.5% TO ABOUT 10% BY WEIGHT OF SOLUBLE  
TUNGSTATE SALT HAVING A PH OF FROM ABOUT  
4.5 TO ABOUT 8.0 AT A TEMPERATURE OF  
FROM ABOUT 130°F. TO BELOW THE BOILING  
POINT OF THE SOLUTION.



FURTHER SEAL THE PARTIALLY SEALED ANODIZED  
OBJECT BY CONTACTING IT WITH AN AQUEOUS  
SOLUTION CONTAINING FROM ABOUT 0.1% TO  
ABOUT 10% BY WEIGHT OF A SALT OF NICKEL  
OR COBALT AND A WEAK ACID AND, IF DESIRED,  
A BUFFERING COMPOUND HAVING A PH OF FROM  
ABOUT 4.5 TO ABOUT 8.0 AT A TEMPERATURE  
OF FROM ABOUT 150°F. TO BELOW THE BOILING  
POINT OF THE SOLUTION.

## PRODUCTION OF STAIN RESISTANT, CLEAR, SEALED ANODIZED FILMS

### CROSS-REFERENCE TO RELATED APPLICATIONS

Geraldine M. Hoch et al. U.S. Pat. application Ser. No. 881,884, filed Dec. 3, 1969 entitled, "Clear Sealing of Anodized Aluminum" assigned to the Lockheed Aircraft Corporation and now abandoned. The entire disclosure of this application is incorporated herein by reference.

### BACKGROUND OF THE INVENTION

The present invention pertains to the sealing of anodized aluminum films so as to improve the corrosion and stain resistance of such films.

It is conventional to anodize aluminum bodies and articles in order to provide upon them adherent, protective aluminum oxide coatings or films. Such coatings or films are normally referred to as anodized coatings or films inasmuch as they are produced by electrolytic processes in appropriate electrolytes at the anodes of electrolytic cells or systems. Normally a sulfuric acid electrolyte is utilized in the production of these anodized films. The oxide coatings produced in this manner are somewhat porous in character and are somewhat subject to various types of corrosion. Further, these anodized films are well recognized to be susceptible to staining as a result of various types of materials contacting these films.

A number of efforts have been made at "sealing" anodized films so as to improve both their corrosion and stain resistance. One such method with which the present invention is particularly concerned is set forth in the aforesaid U.S. patent application Ser. No. 881,884. This method involves contacting a rinsed, anodized aluminum surface with a solution preferably containing from about 1.5 to about 7% by weight of a soluble tungstate salt and from about 0.5 to about 5% by weight of chromic oxide either present as chromic acid or as a soluble salt of this acid having a pH of from about 3.2 to about 8.5 and preferably of from about 5.5 to about 7 at a temperature of from about 150°F. to about 212°F.

Sealed anodized coatings produced in accordance with the process set forth in this co-pending application are considered to be highly desirable because they are substantially clear in character. They are also considered to be highly desirable because of their resistance to corrosion. Parts produced in accordance with the process of this prior application have withstood salt spray testing for significant periods without signs of the usual salt caused corrosion. However, in spite of these advantageous characteristics, sealed anodized coatings produced in accordance with this co-pending application are not considered to be as desirable as reasonably possible for certain commercial applications because they tend to lack adequate resistance to staining.

Normally such resistance to staining is tested on an anodized aluminum article by applying to the surface of such an article a quantity of anthroquinone violet R dye, removing this dye and then determining visually if any of the dye has been absorbed in the anodized coating so as to stain this film or coating. Although a test of this type is subjected to criticism because of its empirical nature, nevertheless this type of test is practical

for determining whether or not an anodized aluminum surface is effectively stain resistant.

The use of this and other related tests has established a need for improvement in the stain resistant character of sealed anodized films produced utilizing a tungstate-chromate bath as indicated. More specifically there is the need for improving anodized coatings sealed with chromates and tungstates so as to retain the advantageous corrosion resistant properties or characteristics produced by such combined sealing and so as to achieve in such coatings an effective, substantially clear stain resistant appearance.

### SUMMARY OF THE INVENTION

An objective of the present invention is to fulfill this need. This invention is intended to provide a new and improved process for sealing anodized coatings which retain the benefits of sealing anodized coatings with tungstate-chromate solutions as indicated, but which also provides in such coatings a degree of stain resistance not achievable with such sealing alone. An objective of the present invention is also to provide sealed, anodized films as indicated. Another objective of the present invention is to provide a process as indicated which may be easily and conveniently carried out at a comparatively minimal cost so that the articles produced by this process can be economically competitive.

In accordance with this invention these and various related advantages of it are achieved by partially sealing a conventionally anodized aluminum body or article by contacting the anodized film on such a body or article with a solution of a soluble tungstate salt and chromate oxide present either as chromic acid or as a soluble salt of it and then subsequently and separately sealing the partially sealed oxide film produced by contacting it with a soluble nickel or cobalt salt of a weak acid. It will be realized that the practice of this invention involves further details than are indicated in this summary.

### BRIEF DESCRIPTION OF THE DRAWING

Such details are conveniently explained with reference to the accompanying drawing in which:

The FIGURE is a flow chart indicating steps in a preferred method of practicing the invention.

This invention, of course, is of an intangible character and is not directly indicated by the accompanying drawing. The features or concepts of this invention are considered to be fully defined or summarized by the appended claims forming a part of this disclosure.

### DETAILED DESCRIPTION

The word "aluminum" employed in this specification is used herein in a broad sense corresponding to the manner in which this word is conventionally utilized industrially. Thus, the word "aluminum" as used herein does not only designate the metal known by this word and/or articles or bodies created from this metal, but it is also utilized to designate alloy compositions and/or articles or bodies created from this metal which are conventionally designated by the word "aluminum" since they predominantly contain this metal. A number of such alloys are commonly known and used. They are frequently designated by trade designations such as 7075-T6, 7075-T76 and 2024-T3 used to designate their composition.

Conventionally such aluminum articles and bodies are anodized in an electrolytic cell or system containing a comparatively strong mineral acid such as sulfuric acid to provide on them a comparatively thick porous film which is physically strong enough to resist normally encountered abrasion and the like. Inasmuch as such anodizing is conventional in the industry it is not considered necessary to describe it in detail in this specification.

It is considered that normally such anodizing is carried out utilizing an aqueous electrolyte containing from about 7 to about 25% and preferably from about 11 to about 17% by weight of sulfuric acid at a temperature of from about 60°F. to about 90°F. and preferably from about 68°F. to about 72°F. at a current density within the range of from about 7 to about 20 amperes per square foot and preferably from about 10 to about 15 amperes per square foot at a voltage normally from about 15 to about 20 volts until an oxide film is produced which is sufficiently thick to withstand the physical abrasion or the like to which it is apt to be subject.

Following such anodization an anodized film may be neutralized in a weak alkaline solution such as a solution containing 5% by weight sodium bicarbonate and then is rinsed. An anodized surface film produced in this manner is well recognized to be somewhat porous in character and to be somewhat susceptible to corrosion of various types and to be susceptible to being stained by contact with a wide variety of different materials.

As set forth in the aforesaid co-pending application such a film can be effectively sealed against corrosion by contacting it with an aqueous solution containing from about 1.5 to about 7% by weight of a soluble tungstate salt and from about 0.5 to about 5% by weight of chromic oxide either present as chromic acid or as a soluble salt of this acid having a pH of from about 3.2 to about 8.5 and preferably of from about 5.5 to 7 at a temperature of from about 150°F. to about 212°F. This process is referred to as "clear sealing" because it produces a clear, corrosion resistant oxide film.

The exact physical and chemical characteristics of a sealed oxide film produced in this manner are not completely known or understood. However, it is believed that in a film of this character tungstate and chromate ions are absorbed into a porous aluminum oxide matrix and are bonded together in the matrix in such a manner as to form a type of an amorphous gel in which all of the oxides are linked together by hydrogen bridges in the form of what may be loosely regarded as a zeolytic type structure in which there are various reactive sites located along an essentially inorganic polymer type structure. Although such sites are considered to be present in an anodized coating which has been "clear sealed" as indicated with a tungstate-chromate bath, such a "clear sealed" coating is advantageous because of economic considerations pertaining to its manufacture, because of its desirable corrosion resistance and because it is of a substantially clear character.

In accordance with this invention it has been found that the corrosion resistance and the stain resistance of such a coating may be improved or enhanced by contacting such a coating with a solution of a soluble nickel or cobalt salt as hereinafter indicated. Such a salt is considered to locate either the nickel or cobalt ion at the reactive sites in an inorganic complex as indicated

so as to in effect block these sites in such a manner that materials which would normally tend to stain an anodized aluminum coating cannot be absorbed or held by such a coating, presumably at these same sites.

5 The effectiveness of the present invention in producing stain resistant as well as corrosion resistant sealed, clear or substantially clear anodized films or coatings is considered to be indicated by what is regarded as a rather significant discovery. This discovery relates to 10 the fact that effective stain and corrosion resistant sealed films can be created in which this step of treatment with a nickel or cobalt ion is preceded by a "clear sealing" process as indicated carried out utilizing a solution containing smaller quantities of both tungstate and chromate ions than previously considered necessary in "clear sealing". This is considered important because it permits lesser quantities of materials to be used in making up solutions to be utilized with a two-step process as herein described than one would normally consider necessary then if the present invention merely 15 added an additional step to prior "clear sealing".

In accordance with this invention an initial "clear sealing" operation can be carried out utilizing an aqueous solution containing from about 0.1% to about 5% by weight of chromic oxide either present as a chromic acid or as a soluble salt of this acid and from about 0.5% to about 10% by weight of soluble tungstate salt having a pH of from about 4.5 to about 8.0 at a temperature of from about 130°F. to a temperature immediately below the boiling point of the solution. Certain specific aluminum compositions are considered to be 20 most effectively sealed using ranges and proportions within the limits given which are determined empirically with reference to the corrosion resistance achieved.

25 It is noted that the proportions of such ingredients given in these ranges are lower than those given in the preceding discussion relative to "clear sealing". It will also be noted that the temperature range useable with 30 this invention during this initial partial sealing step is somewhat different than the temperature range indicated in the preceding as required for effective "clear sealing". Further, there is a minor difference in the pH of the solution used in this initial "clear sealing" operation. These differences are considered to point out the 35 fact that the initial "clear sealing" used with the invention need only be what can be regarded as a partial sealing.

The bath used in this initial sealing can easily be created utilizing a conventional soluble tungstate salt such 40 as a potassium, sodium, lithium or ammonium salt. It is also possible to utilize potassium, sodium or ammonium metatungstates or a combination of any of these salts. The chromate used may be in the form of chromic 45 trioxide (which of course forms chromic acid in solution) or a conventional chromate compound such as a sodium, potassium, lithium or ammonium chromate or dichromate or any mixture of these. This initial sealing solution should consist essentially of these salts 50 in the sense that it should contain only a mixture of one or more tungstates and one or more chromates and if reasonably necessary, a suitable pH adjusting compound such as sodium hydroxide or the like containing ions such as alkali metals ions and hydroxide ions which will not significantly enter into the sealing action obtained, and, if desired one or more conventional wetting agents used in accordance with conventional practices.

tice so as to facilitate solution penetration into an anodized surface provided that such a wetting agent is of a known type not effecting the sealing action obtained.

The proportions of the tungstate (s) or chromate (s) used in the bath in this initial partial sealing are primarily dictated by practical considerations. If amounts of either of these two types of ions below those indicated are present in the sealing solution a partially sealed anodized film having less than a desired degree of corrosion resistance will be achieved. On the other hand, if greater amounts than are indicated are used, there tends to be an uneconomic or unnecessary use of material.

A pH within the range indicated is preferred during this initial sealing since a lower pH than 4.5 may result in some acidic-type attack on the aluminum treated and/or on the oxide film present on this aluminum. With higher pH's than are indicated there is also the possibility of alkaline attack on the aluminum and the oxide. When solution temperatures below the 130°F. figure are used it appears that a desired partial type seal action is not effectively obtained. If a maximum temperature of the sealing solution is used which corresponds to the boiling point of this solution the vaporization of water may tend to interfere with the formation of a uniform, at least partially sealed coating.

Although as indicated the "clear sealing" step carried out in accordance with this invention may be performed utilizing various broad ranges of ingredients and conditions as indicated, it is preferred to carry out the invention utilizing the more specific ranges and conditions indicated in the preceding discussion as to prior, known "clear seal" process of sealing utilizing a combined tungstate-chromate bath. This is because it is considered that it is advisable to seal an anodized coating as completely as possible in the initial sealing step so as to avoid any chance of such a coating being completely sealed because of failure of any type of the secondary sealing operation performed in accordance with this invention. In essence, however, this is a matter of choice.

This initial sealing step or partial sealing step in accordance with this invention can be carried out in accordance with conventional practice by either dipping an article to be sealed in a bath as specified or by spraying such a bath on such an article. The time of contact between this initial "clear sealing" solution will, of course, effect the completeness of the sealing accomplished during the treatment with it. It is considered that effective sealing can be accomplished with a contact period of at least one minute. Preferably, however, the contact time between an article being partially sealed in the solution should be longer in order to make sure that there is adequate, reasonably complete partial sealing during this step. It is considered that if a time period in excess of about twenty minutes is used that nothing is gained as a result of the use of this long a period. In general, the hotter the temperature of the sealing solution used the lower the time period required.

An anodized film or coating at least partially sealed with a tungstate-chromate bath as indicated in the preceding is further sealed in accordance with this invention with a solution containing from about 0.1 to about 10% by weight of a soluble nickel or cobalt salt. In general, the lower the concentration of such a bath, the

less effective it is in providing adequate stain resistance while if a solution is used having a higher concentration than indicated, significant benefit in sealing is observed.

It is considered significant that the nickel or cobalt salt used with the present invention should be a salt of a weak acid such as the salt of either of these metals and an acid selected from the group consisting of boric acid, citric acid, formic acid and acetic acid. Salts of these metals with other acids than are indicated are considered to normally impart to a sealed anodized film as herein described a degree of color rendering an anodized, sealed film as herein indicated unacceptable for certain applications where a substantially clear, colorless film is required. Mixtures of various salts as indicated can be employed with the present invention.

When this second sealing solution has a pH below about 4.5 it is considered that there is a tendency for the acidity of this solution to attack the aluminum being treated with it and/or the treated oxide film on the aluminum. When the pH of this secondary treatment solution is relatively high such as at a pH of 8 or above, it is considered that there is normally a problem of maintaining a desired, effective concentration of the salt used. This is because nickel and cobalt salts as employed tend to precipitate out at relatively high pH's. Indeed, with certain salts there can be solubility problems at even pH's below this pH of 8. Because it is considered that an acidic pH tends to promote the formation of the type of complex believed to be created by practicing the present invention, it is normally preferred that this secondary treatment solution employed have a pH of no greater than 7.

The importance of pH in this secondary, final sealing is considered to make it desirable to buffer the solution used in accordance with conventional practice so that this solution will have a constant pH or a substantially constant pH within the range of from about 5.5 to about 6.5. This ultimate treatment solution can be conveniently buffered to within this pH range through the use of one or more of the enumerated acids and/or through the use of salts of such acids which do not effect the sealing action achieved. Thus, acids such as boric acid, citric acid, formic acid, acetic acid and salts of such acids such as the sodium, lithium and ammonium salts of these acids can conveniently be utilized for buffering purposes. The amount of such a buffering reagent should of course, be determined on the basis of conventional considerations.

In order to avoid the possibility of secondary ingredients interfering with this secondary sealing step, it is preferred that the solution used consist essentially of only one or more of the nickel or cobalt salts indicated or consist essentially of one or more of such salts and one or more buffering reagents as described. Thus, the treatment solution used should be free from metallic ions other than alkali metal ions and from acidic ions other than those of the acids specifically enumerated. If desired the solution used may contain one or more conventional wetting agents used in accordance with conventional practice so as to facilitate solution penetration provided that such a wetting agent is of a known type not affecting the sealing action obtained. Suitable wetting agents may be anionic, cationic, or nonionic and may be conveniently used in amounts up to about 3% by weight of the solution.

Substantially the same considerations as specified in the preceding regarding the temperature of the "clear sealing" solution govern the temperature of the solution during this final sealing step. In general, if temperatures below about 150°F. are used, the sealing accomplished tends to be inadequate. If a temperature at or above the boiling point of the solution is employed there is a possibility that a uniform sealing action will not be achieved due to the vaporization of water.

In general, the higher the temperature required the less the time with which the bath need be in contact with the film or coating being processed. Contact periods of from one to twenty minutes are normally considered satisfactory. If the contact time is less than this there is a danger that there may be inadequate sealing. On the other hand, if periods greater than about twenty minutes are used no significant benefits are achieved. In general, the higher the salt concentration of the secondary sealing solution the less the time required.

This secondary sealing step may also be carried out by either dipping or immersing an at least partially "clear sealed" article as indicated in a bath as specified in the preceding or by spraying such solution on to an at least partially sealed oxide film or coating as indicated so that there is contact between the film and coating and the solution for a time period and at a temperature as specified.

The fact that this secondary sealing achieves an unexpected type reaction and/or series of reactions is considered to be illustrated by the colorless character of a final sealed film produced. As indicated in the preceding this is important for commercial reasons. This unexpectedness is indicated by the fact that nickel and cobalt chromates and tungstates normally possess a distinct color. Thus, for example, nickel chromates are of a brown color and nickel tungstates are of a greenish type color. The absence of these colors in films sealed with nickel salts as indicated indicates that these compounds are not formed as a result of a final sealing step as herein described.

The following examples are given as an aid to understanding the present invention. It is understood that these examples are given for this purpose only. They are not to be considered as limiting the invention in any respect.

#### EXAMPLE 1

A test panel of 7075-T6 aluminum material anodized in a sulfuric acid electrolyte in accordance with conventional practice can be partially sealed by immersing it in an aqueous solution containing 5% by weight sodium tungstate and 1% by weight chromic acid having a pH of 6.5 at a temperature of 200°F. for about 10 minutes. This panel can then be further sealed by immersing it in a solution containing about 1% by weight nickel acetate at a temperature of about 200°F. for a further period of 10 minutes. At the end of this period the panel can be dried and used in accordance with conventional practice.

#### EXAMPLE 2

A test panel of 7075-T76 aluminum material anodized in a sulfuric acid electrolyte in accordance with conventional practice can be partially sealed by immersing it in an aqueous solution containing 7% by weight sodium tungstate and 3% by weight chromic oxide at a temperature of about 140°F. for a period of

15 minutes. Immediately following this the panel can be further sealed by immersing it in a solution containing about 3% by weight nickel acetate and 4% by weight boric acid at a temperature of about 160°F. for a period of about 3 minutes.

It would be possible to multiply these examples almost indefinitely by varying the specific salts, concentrations and other details set forth in them so as to recite in specific example form all of the parameters of 10 the invention indicated in the preceding discussion. Inasmuch as the invention is relatively simple it is believed that no useful purpose would be achieved by such enlargement of this specification. The important thing is that effectively stain resistant, sealed anodized 15 aluminum oxide coatings can be easily and conveniently produced at a comparatively nominal cost as described in this specification.

We claim:

1. In a process of sealing an anodized aluminum coating in which said coating is contacted with a first solution containing tungstate and chromate ions so as to partially seal said anodized coating, the improvement which comprises:

25 contacting the anodized coating which has been contacted with said first solution after it has been removed from said first solution with a further solution containing from about 0.1% to about 10% by weight of a soluble salt of a metal selected from the group consisting of nickel and cobalt and of a weak acid at a temperature of from about 150°F. to immediately below the boiling point of said solution for a period sufficient to further seal said anodized coating in order to render said anodized coating substantially stain resistant.

2. A process as claimed in claim 1 wherein: said further solution consists essentially of water and said salt and said weak acid is an acid selected from a group consisting of boric, citric, formic and acetic acids.

3. A process as claimed in claim 1 wherein: said further solution consists essentially of water, said salt and a buffering compound, and said weak acid is an acid selected from a group consisting of boric, citric, formic and acetic acids, and

40 said buffering compound is a compound selected from the group consisting of boric acid, citric acid, formic acid and acetic acid and ammonium and alkali metal salts of such acids.

4. A process as claimed in claim 1 wherein: said further solution contacts said anodized coating for a period of from about 1 to about 20 minutes and has a pH of from about 4.5 to about 8.

5. A process as claimed in claim 1 wherein: said first solution consists essentially of water and from about 0.5 to about 10% by weight of a soluble tungstate salt, from about 0.1 to about 5% by weight chromic oxide present as chromic acid or as a soluble chromate salt, has a pH of from about 4.5 to about 8 and is in contact with said anodized coating for a period of from about 1 to about 20 minutes at a temperature of from about 130°F. to immediately below the boiling point of said solution,

60 said further solution is a solution selected from the group consisting of (1) aqueous solutions consisting essentially of said salt and of (2) buffered aque-

ous solutions consisting essentially of said salt and a buffering compound, said weak acid being selected from the group consisting of boric, citric, formic and acetic acids, said buffering compound being selected from the group consisting of boric acid, citric acid, formic acid and acetic acid and ammonium and alkali metal salts of such acids, said further solution having a pH of from about 4.5 to about 7 and contacting said anodized coating for a period of from about 1 to about 20 minutes. 5

6. A process as claimed in claim 5 wherein: the pH of said further solution is from about 5.5 to about 6.5.

7. A process as claimed in claim 5 wherein: said first solution includes a wetting agent serving to 15 facilitate penetration of said first solution into said anodized coating.

8. A process as claimed in claim 5 wherein: said further solution includes a wetting agent serving to facilitate penetration of said further solution into 20 said anodized coating.

9. A process as claimed in claim 5 wherein: both of said first and said further solutions include a 25 wetting agent serving to facilitate penetration of said solutions into said anodized coating.

10. An anodized, sealed aluminum oxide coating produced by the process of claim 5.

11. A process for sealing an anodized aluminum coating which comprises:

contacting said coating after it has been anodized and 30 before it has been further sealed for a period of from about 1 minute to about 20 minutes with a first solution containing essentially water and from about 0.1% to about 5% by weight chromic oxide present as a compound selected from the group 35 consisting of chromic acid and soluble chromate salts and from about 0.5% to about 10% by weight of a soluble tungstate salt, said solution having a pH of from about 4.5 to about 8.0 and being at a temperature of from about 130°F. to immediately 40

below the boiling point of said solution, and thereafter directly contacting said anodized coating for a period of from about 1 to about 20 minutes with a further solution selected from the group consisting of (1) solutions consisting essentially of water and from about 0.1% to about 10% by weight of a salt of a metal selected from the group consisting of nickel and cobalt and of an acid selected from the group consisting of boric, citric, formic and acetic acids and (2) solutions consisting essentially of water and from about 0.1% to about 10% by weight of a salt of a metal selected from the group consisting of nickel and cobalt and of an acid selected from the group consisting of boric, citric, formic and acetic acids and of a buffering compound selected from the group consisting essentially of boric, citric, formic and acetic acids and ammonium and alkali metal salts of such acids, said further solution having a pH of from about 4.5 to about 8 and being at a temperature of from about 150°F. to immediately below the boiling point of said solution.

12. A process as claimed in claim 11 wherein: said further solution has a pH of from about 5.5 to about 6.5.

13. A process as claimed in claim 11 wherein: said first solution includes a wetting agent serving to facilitate penetration of said first solution into said anodized coating.

14. A process as claimed in claim 11 wherein: said further solution includes a wetting agent serving to facilitate penetration of said further solution into said anodized coating.

15. A process as claimed in claim 11 wherein: both of said first and said further solutions include a wetting agent serving to facilitate penetration of said solutions into said anodized coating, said further solution has a pH of from about 5.5 to about 6.5.

\* \* \* \* \*